

# UNITED STATES PATENT OFFICE.

RUDOLF SILBERBERG, OF JERSEY CITY, NEW JERSEY, ASSIGNOR OF ONE-HALF TO HENRY W. HOOPS, JR., OF SAME PLACE.

## MORDANT.

SPECIFICATION forming part of Letters Patent No. 320,821, dated June 23, 1885.

Application filed May 8, 1885. (No specimens.) Patented in Canada April 20, 1885, No. 21,458.

*To all whom it may concern:*

Be it known that I, RUDOLF SILBERBERG, a citizen of the United States, residing at Jersey City, in the county of Hudson and State of New Jersey, have invented certain new and useful Improvements in Mordants, of which the following is a specification.

My invention is an improved mordant of a character to deposit chromium oxide upon cotton and other fabrics in order to adapt the same to be dyed fast-colors by the use of aniline dyes.

In the preparation of my mordant I use oxalate of chromium, which I prepare in the following manner: I first dissolve sixty-six pounds of bichromate of potash in ninety-three pints of boiling water, and add to the solution fifty-five pints of nitric acid of a strength of 36° Baumé. I then prepare a second solution of twenty-nine pounds of oxalic acid in sixty pints of water, and add sixteen pints of glycerine of a strength of 28° Baumé. The two solutions are added together and boiled until a diluted solution appears of a clear green color, after which the solution is allowed to stand until nitrate of potash is deposited as crystals, when the oxalate of chromium will be in solution in the liquor of a strength of 35° to 38° Baumé.

In making the mordant I take twenty quarts of the above-mentioned liquor diluted with water to 8° Baumé, and mix therewith seven-

teen and a half quarts of a solution of caustic soda of a strength of 20° Baumé, and after the two are well mixed I add five quarts of 35 water.

The mordant mixture thus produced constitutes a salable preparation.

When the mordant is to be used for mordanting fabrics, a portion thereof is diluted with double its volume of cold water, and the goods, after being soaked in boiling water, are soaked in the mordant-liquor for ten hours, and then removed, thoroughly washed, and dyed in the ordinary manner.

I do not here claim the mode of making an oxalate of chromium or the mode of dyeing aniline colors therewith, as the same constitutes the subject of separate applications for Letters Patent Nos. 160,074 and 160,075.

I claim—

A mordant for preparing fabrics for dyeing with aniline dyes, consisting of a mixture of a solution of oxalate of chromium and a solution of caustic soda, substantially as described.

In testimony whereof I have signed my name to this specification in the presence of two subscribing witnesses.

RUDOLF SILBERBERG.

Witnesses:

FRANK J. MATHEWS,  
HENRY W. HOOPS, Jr.